

Jan. 19, 1932.

W. E. GREENAWALT

1,841,437

COPPER EXTRACTION PROCESS

Filed Nov. 9, 1926



INVENTOR.

William E. Greenawalt.

## UNITED STATES PATENT OFFICE

WILLIAM E. GREENAWALT, OF DENVER, COLORADO

## COPPER EXTRACTION PROCESS

Application filed November 9, 1926. Serial No. 147,324.

The process has as its object the production of electrolytic copper from its ores without resorting to regular smelting and refining methods, which, in most mining districts, are too expensive for general adoption, especially in small or medium sized units.

The following considerations are the principal factors governing the process, and when these are understood the process can be easily comprehended.

The two outstanding difficulties in the treatment of high grade copper ore or concentrate by leaching and electrolysis are, first: the formation of ferrites and ferrates in roasting, which results in high tailing loss on leaching, and second: the solubility of iron and other impurities, which are always dissolved with the copper and which cause trouble in leaching and in the electrolytic deposition of the copper from the impure copper solutions. These difficulties can be minimized, but it is thought that the present process presents advantages in this direction, over the usual methods.

Most mines, or mining districts, produce large amounts of low grade copper ore, usually in the form of sulphide, or as the sulphide and oxide (including carbonate and silicate) mixed. In either case the general method of procedure is to separate the sulphide mineral from the gangue to form a concentrate. This concentrate is usually of relatively low grade, as compared with the theoretical percentage of copper in the mineralogical combination of the copper minerals. Considerable gangue is associated with the copper in the concentrate, and usually a large amount of iron, either as pyrites, or combined mineralogically with the copper, as in bornite or chalcopyrite. Quite frequently chalcocite, having the mineralogical formula of  $Cu_2S$ , will form a constituent of the various copper ores, and to some extent also covellite, which has the mineralogical formula of  $CuS$ .

In the concentration treatment of copper ores, the concentrate is usually so contaminated with iron, silica, alumina, etc., that vigorous fluxing is required for good smelting conditions, and this makes a smelting

process expensive to install and expensive to operate. Where power is cheap and fuel is costly, electric smelting would appear to offer some advantages, but the complications arising from the fluxing of large quantities of material and the large amount of electricity required, has led to failure or disappointment wherever it has been tried.

In the concentration treatment of mine ore, either by gravity or flotation, a certain amount of very high grade concentrate may be separated from the large amount of the ordinary sulphide concentrate, but the relatively small amount of very high grade concentrate will contain a relatively large portion of the total copper. Usually this relatively small portion of high grade concentrate will be in the form of the practically pure minerals, chalcocite, bornite, and chalcopyrite. Pure chalcocite contains 79.8% copper and 20.2% sulphur; pure bornite contains 55.8% copper, 28.6% sulphur, and 16.36% iron; pure chalcopyrite contains 34.6% copper, 34.9% sulphur, and 30.5% iron.

The conditions of concentration can best be illustrated by taking a specific case in the treatment of 100 tons of ore assaying 1.5%, or 30 pounds, of copper per ton, or containing a total of 3,000 pounds of copper. If the ratio of concentration is 10 into 1, we would have, as the result of the concentration treatment:

90 tons tailing, 0.25% copper (5 lbs.), 450 lbs. total.

10 tons concentrate, 12.75% copper (255 lbs.), 2550 lbs. total.

The ten tons of concentrate may be separated into:

1.5 tons high grade concentrate, 50% copper (1000 lbs.), 1500 lbs. total.

8.5 tons low grade concentrate, 6.2% copper (124 lbs.), 1050 lbs. total.

There should not be any great difficulty under most conditions to get a 50% copper concentrate in the relatively small amounts indicated, if much of the copper in the ore is in the form of chalcocite or bornite, and

this is usually the case in what are known as porphyry, or disseminated, deposits. It will be understood, however, that the process is not particularly limited to the percentage of 5 copper in the high grade concentrate, but that the higher the grade of the high grade concentrate, the better the process can be operated as a whole.

Having made the separation of the mineral 10 from the gangue and divided the mineral into a relatively small amount of high grade concentrate and a relatively large amount of low grade concentrate, the method of procedure is as follows, reference may be made 15 to the accompanying drawing which is a flow sheet of the process, in diagrammatic plan.

The relatively small amount of high grade 20 concentrate, which according to the specific case assumed for illustration purposes will consist of 1.5 tons of 50% copper concentrate per 100 tons of original ore, is roasted so as to make as much as practical of the copper water soluble and a high percentage soluble in dilute acid. By careful roasting, from 25 80% to 85% of the copper can be made soluble in water and from 85% to 97% soluble in dilute acid.

When copper ore or concentrate is roasted 30 so as to make a large portion of the copper water soluble, some iron is also made soluble, but the amount of water soluble iron is small as compared with the acid soluble iron.

The roasted high grade concentrate is transferred to the leaching tank No. 1, where 35 it is leached, preferably first with water and then with dilute acid, although the acid leach may at times be dispensed with to advantage, especially when the water soluble copper is exceptionally high.

The roasted high grade concentrate is 40 leached with water or very dilute acid, which will extract from 80% to 85% of the copper, and the resulting copper sulphate solution will be quite pure, altho it will contain small amounts of iron and other impurities, but not 45 in sufficient amounts to seriously affect the subsequent electro deposition of the copper.

The copper solution flows from the leaching 50 tank No. 1 into the settler No. 1. This settler may also act as a storage tank. It may also act as a reducer for ferric iron, when the solution is treated with copper sulphide. High grade copper sulphide for this purpose 55 may be obtained from the original ore, by fusion, or as CuS precipitate obtained in treating lean and foul solution with hydrogen sulphide.

The copper solution flows into the copper 60 tanks No. 1, where the copper is deposited as electrolytic copper of great purity, with the simultaneous regeneration of acid. Owing to the small amount of injurious impurities in the electrolyte, the solution can be fairly impoverished in copper and regenerated in acid. 65 It may then be transferred to the low grade

concentrate leaching and electrolytic circuit. A portion of it may be returned to the roasted high grade concentrate leaching tank No. 1. If the solution issues from the leaching tank No. 1, containing, say 8% or 10% copper, and containing only a small amount of iron, it is quite practical to impoverish the solution down to about 2% copper, with a very high ampere efficiency. It is preferred 70 to deposit most of the copper in the copper tanks No. 1, from a rich copper solution, which will result in the best possible copper and the highest ampere efficiency obtainable under the conditions, and then pass the impoverished solution to copper tanks No. 2, where the copper may be reduced to the desired extent, say, to 1% or less. This solution, low in copper and high in acid is then passed to the low grade concentrate leaching 75 and electrolytic circuit.

The relatively large amount of low grade 80 concentrate, which according to the specific case assumed for illustration purposes will consist of 8.5 tons of 6.2% copper concentrate, per 100 tons of original ore, is roasted so as to make as much copper water soluble as practical, and a high percentage soluble in dilute acid. From 75% to 85% of the copper can be made water soluble by careful roasting, and from 85% to 97% can be made acid soluble. 85

It is preferred to add the leached tailing 90 from the high grade concentrate to the low grade concentrate, and roast the mixture. This means a double roasting for the high grade concentrate, but since the amount of high grade concentrate residue is very small and will usually contain copper worth recovering, this method of procedure offers evident 95 advantages. The residue will be only a half or a third of the original high grade concentrate. The extraction by double roasting of the high grade concentrate, can be made almost complete, or at least give a final residue as low in copper as the residue resulting from leaching the roasted low grade concentrate. The extraction may be as high as 97% to 99% 100 of the original copper in the high grade concentrate, as set forth in some detail in my Patent No. 1,468,806, Sept. 25, 1923.

The roasted low grade concentrate is, preferably, first leached with water or very dilute acid solution, in leaching tank No. 2, and the rich water soluble copper solution is flowed 105 into the water CuSO<sub>4</sub> storage tank. The water soluble copper solution will be practically neutral and contain very little iron, as described for the high grade concentrate. If, however, there should be more iron in the water soluble copper solution than desired, the solution may be treated with high grade 110 copper oxide, obtained from roasting high grade concentrate. The water soluble copper solution is transferred to the high grade concentrate leaching and electrolytic circuit, 115 preferably by using it as the leach water so- 120

lution for the roasted high grade concentrate. This will give a very rich and a quite pure neutral copper sulphate solution, and the amount of water used will be reduced to a minimum. With care in leaching, a large portion of the iron may be precipitated from the water soluble copper solution with the high grade roasted concentrate, and when the residue is roasted, the precipitated iron will be made insoluble. The water soluble copper solution obtained by first leaching the roasted low grade concentrate and then the roasted high grade concentrate, is then electrolyzed to deposit the copper and regenerate acid, as described for the copper sulphate solution obtained by water leaching the high grade concentrate. Copper sulphate is quite soluble in water. At 70 deg. C., which would be a fair temperature of the water in leaching hot roasted concentrate, a water saturated solution of copper sulphate will contain 12.93% copper, and there should be no difficulty in keeping the head solution for copper deposition at from 8% to 10% copper, in leaching the roasted concentrate as described. Such a rich copper solution is not necessary, nor may it be desired, but it is obtainable, if desired.

The regenerated acid solution, resulting from the deposition of the copper from the relatively pure water soluble copper solution, is quite free from injurious impurities. A portion of this acid solution may be added to the water, for the water soluble copper solution in amount so that the acid will be quickly neutralized by the copper in the roasted concentrate, which is insoluble in water. This copper will be mostly in the form of oxide. Iron is not readily soluble in a weak acid solution, but, at the same time, the copper oxide in the roasted concentrate will be quickly dissolved in a weak acid solution. It is practical, therefore, to leach out the larger portion of the readily soluble oxide of copper with a very weak acid solution, without appreciably increasing the iron content of the solution, and, as already indicated, if the iron occurs in the solution in undesirable amounts, it can easily be precipitated from the neutral solution with an excess of concentrated copper oxide. The precipitated iron in the high grade concentrate residue can be made insoluble by roasting the residue with the low grade concentrate. It should be practical, in this way, to extract 80% of the copper from the roasted low grade concentrate and 95% of the copper from the roasted high grade concentrate, without appreciably fouling the solution.

If the extraction of the copper from the roasted high grade concentrate is 95%, and the loss of weight by roasting and leaching is 60%, the high grade concentrated leached residue will still contain about 6.25% copper. Much of this copper in the residue can be

extracted with strong acid, and the resulting highly impure solution transferred to the low grade concentrate leaching and electrolytic circuit, but ordinarily this extra leaching of the roasted high grade concentrate may be dispensed with and the residue obtained from leaching with water or very dilute acid solution may be added to the low grade concentrate and roasted with it. With the re-roasting and re-leaching of this high grade leach concentrate residue the extraction will be almost complete.

Washwater, or lean water soluble copper solution, resulting from leaching of one charge of either the roasted high grade or low grade concentrate, may be used as the head solution for another charge.

It will be noticed that, water leaching, or very dilute acid leaching, so as to obtain neutral, or practically neutral solutions, an amount of water, or regenerated acid solution, is discarded, equal to the amount of water added, and that in this way the injurious impurities in the rich, or water soluble copper solution, may always be maintained so low as not to give any serious leaching or electrolytic difficulties.

After the roasted low grade concentrate has been leached with water or with very dilute acid solution as described, it is leached with the regenerated acid solution obtained from depositing the copper from the water soluble copper solution. This strong acid solution will be usually quite impure. It will contain the relatively small amount of impurity from the water soluble copper leaching and electrolytic circuit, and the relatively large amount of impurity resulting from leaching the roasted low grade concentrate with the relatively strong acid solution. The strong acid solution will dissolve the copper in the roasted low grade concentrate which was not soluble in water, or very dilute acid, and if the total extraction is 95% the leached roasted low grade residue will contain about 0.31% copper, based on the weight of the original concentrate.

The impure solution, containing salts of iron and other impurities, flows into the settler, or reducer No. 2, where it may be clarified and treated with copper sulphide to reduce ferric iron to ferrous iron. The solution then flows into the  $\text{SO}_2$  reducer, and from the reducer into the storage tank, and from the storage tank into the copper tanks No. 3, where the copper is deposited and acid and ferric iron regenerated. A portion of the solution is returned to the roasted low grade concentrate and the cycle repeated until the copper in the roasted low grade concentrate is sufficiently extracted, as described more in detail in my Patent No. 1,483,056, Feb. 5, 1924, and another portion, the excess, may be wasted, or, if the original ore contains copper in oxidized form, such as

the oxide, carbonate, or silicate, the excess may be used to leach the oxidized copper from the original ore, or from the concentrator tailing, preferably as will now be described.

The ore, which may be presumed to be crushed to about  $\frac{1}{4}$  inch in the primary crusher, is fed into the rod mill, where it is ground to, say, 48 mesh, which may be presumed to be the fineness required for the effective flotation or gravity concentration of the sulphides, as determined by experimentation. A rod mill is preferred for fine grinding, since that will require the least amount of water and have the least amount of returned oversize, and consequently a small circulating load, and this oversize can be kept fairly low, even as low as 25% and lower, without appreciably reducing the efficiency of the rod mill.

When the finely ground ore pulp, containing, say, about 25% water, issues from the rod mill, it is mixed with about three times the amount of acid solution produced by leaching and electrolysis in the treatment of the concentrate as described. This will give about the right proportion of liquid to solids for the classification to 48 mesh. This acid pulp then flows into the classifier where the acid solution acts upon the oxidized copper in the ore to dissolve it, while at the same time a classification is made to 48 mesh. The minus 48 mesh passes to the copper solution separator, and the oversize is returned to the rod mill for re-grinding.

In order to avoid injurious effects of acid and soluble copper in the rod mill, the oversize is washed to free it from acid and soluble copper, and this can be conveniently done, at least in part, by washing the oversize with a slightly alkaline solution and containing a precipitant for the small amount of copper in the washed oversize. This step is easily and cheaply carried out, and with the exception of this step, the grinding and classification is about the same as grinding and classification with ordinary water. The precipitated copper from washing the oversize in regrinding is re-dissolved in the classifier. The operation of grinding the ore and its classification and leaching in an acid solution can be made clear by assuming a specific case. Suppose the grinding in the rod mill is done so that there will be a return of 25% oversize. This will not greatly reduce the efficiency of the rod mill from its maximum, and the extra cost of grinding, as compared with a normal oversize return of from 40% to 50%, will be nominal. With a 25% oversize return, there would be 500 pounds of oversize per ton of ore fed to the rod mill. The water or dilute acid solution of this oversize in the upper portion of the classifier, would be about 20%, or 100 pounds of solution, for the 500 pounds of oversize,

or about 1.3 pounds of acid and 1.3 pounds of copper, per ton of ore ground to the desired fineness to pass the classifier, assuming the acid content of the solution in the classifier after treating the ore, at 1.0%, and the copper content at 1.0%. 1.3 pounds of acid would therefore have to be neutralized and 1.3 pounds of copper would have to be precipitated, per ton of ground ore, assuming that the oversize is not washed at all. If, however, the oversize is water washed in the upper portion of the classifier, so as to displace acid solution with water, most of the acid and most of the copper can be washed from the oversize, depending on the amount of the washing. The washing can be made practically complete, but this might add too much water to the classifier and thus undesirably dilute the acid solution. But if only about enough water is added to the upper portion of the classifier to displace most of the acid and copper in the oversize, no appreciable amount of water will be added to the acid solution in the classifier. The acid and the copper in the oversize, as it is discharged from the classifier into the washer, may be reduced to about 25%, or about 0.25 pound to 0.5 pound of acid and of copper, per ton of ore ground. This amount of acid is easily neutralized and this amount of copper is easily precipitated in the washer, by washing with a dilute alkaline solution containing a precipitant for the copper. A small amount of flotation agent may be added to the washer to overflow a portion of the precipitated copper in the washer, into the classifier. The small amount of acid can also be quickly neutralized by mixing the oversize with new ore to be ground, so that the process is not a delicate one, and can be carried out at a very nominal extra expense over ordinary wet grinding, and much cheaper than dry grinding to the same fineness.

It is preferred to separate the richer portion of the copper solution from the ore pulp, in the copper solution separator, but without attempting to separate all of the soluble copper from the pulp, by excessive washing. The richer impure copper solution, without filtering or unnecessary clarification, is treated a precipitant for the copper, preferably with hydrogen sulphide, by means of which the copper is precipitated as copper sulphide with a regeneration of an equivalent of acid. The mixture of solution and precipitate flows into the CuS separator, where the CuS is separated from the acid solution. The CuS may be added to the high grade concentrate and roasted, or a portion, or all of it, may be used as a reducing agent for ferric iron produced in the deposition of the copper. The barren acid solution may be wasted, or a portion of it may be returned to the classifier for reuse.

Since the larger portion of the copper in

both the roasted high grade and low grade concentrate is soluble in water, and since an equivalent of acid is regenerated from the water soluble copper, as well as a certain amount from the acid soluble copper, the copper in the original ore, in the form of oxide, can be leached out without any acid expense. If, for example, 80% of the copper in the roasted concentrate is water soluble, or about 2040 pounds of the total 2550 pounds in the concentrate, an abundance of acid will ordinarily be regenerated to dissolve, say, 70% of the assumed 0.25%, of the oxidized copper in the original ore, or about 310 pounds. That is to say, there will be about seven times as much acid regenerated in depositing about 2550 pounds of copper obtained from the concentrate, as that theoretically required to dissolve the 310 pounds of copper in oxidized form from the original ore, and this will provide an abundance of excess acid to react with the base elements in the original ore. The precipitated copper sulphide will, however, be quite free from injurious impurities.

The leached ore, from the copper solution separator, without excessive washing, or still containing a small amount of soluble copper, is treated with a precipitation agent for the copper, preferably a sulphide precipitation agent, such as hydrogen sulphide, to precipitate the copper. If the solution is to be made neutral or slightly alkaline, a small amount of caustic lime or caustic soda may be added to the leached ore, as it goes into the concentrator, where the sulphide copper concentrate is separated from the gangue, either by gravity or flotation or by both combined. The CuS precipitate will be floated with the other sulphides in the ore and form part of the high grade concentrate. The tailing may be wasted.

In electrolyzing the rich water soluble copper solution as described, a fairly high acid solution will be regenerated, and, as this high acid solution may advantageously be diluted for leaching the oxidized copper, it can conveniently and profitably be done by grinding the ore wet and simply adding the acid solution to the wet ground ore to give the pulp the consistency for the desired classification.

In most mixed ores, that is to say, ores containing the copper both as the oxide and the sulphide, the sulphide is frequently coated with an oxidized (usually carbonate) film. The oxide in the ore is usually the result of the oxidation of the sulphide, and while much of the oxide (including carbonate) coating may be removed by grinding, nevertheless, it cannot be so perfectly removed as not to present a serious difficulty in many, or most cases for the best conditions for flotation. If, on the other hand, the oxidized portion of the copper in the ore is first removed by a solvent process, the sulphide copper is fully exposed

and the best conditions are obtained for successful flotation, with the consequent highest total extraction of the copper, both in its oxide and sulphide combinations. Leaching before flotation presents certain decided advantages over leaching after flotation, among which is usually a higher total extraction of the copper, and the process, as a whole, is greatly simplified.

Where leaching precedes flotation, or constitutes the entire process, the ore is practically always crushed dry. Dry grinding, with the accompanying screening, is expensive and quite a nuisance if the grinding is fine for flotation. Fine dry grinding of low grade copper ores is rarely, if ever, attempted for leaching only.

Wet grinding is much to be preferred, because it is cheaper than dry grinding, and the screening and dust nuisances are avoided. The difficulty in wet grinding and subsequent leaching, however, arises that the water necessary for wet grinding and classification has to be eliminated to avoid undue dilution and waste of the solvent, and it is quite impractical to dewater the ore pulp much below 50% without filtering, and filtering is too expensive in the treatment of low grade ores. Then, again in the usual conditions of operation large quantities of wash water have to be applied to the acid leached residues to recover the soluble copper. The loss of acid by this excessive addition of water, and the precipitation of the copper from the large volumes of wash water present serious economic problems.

Ordinarily the cost of acid required for leaching presents a serious problem in copper mining districts. In small leaching installations an acid plant would be too expensive to install and to operate. Acid could not ordinarily be delivered in any ordinary mining district for less than about \$20 per ton, and even if manufactured on the ground the cost would be about \$10 per ton. This acid cost is avoided by the present process, and the acid expense for leaching is practically nothing. It is highly desirable also that all of the copper should be obtainable as the electrolytic metal, salable direct to the consumer, to avoid excessive transportation and refining charges. This, too, is realized in the present process.

If a portion of the foul solution obtained from leaching the original ore can be regulated so as to obtain sufficient copper for effective electrolytic deposition or precipitation, it is preferred to precipitate it that way, as being easier and cheaper than hydrogen sulphide precipitation. It will usually be quite practical to get a sufficiently rich copper solution from the large tonnage of original ore to make this step advisable. It will also usually be desirable to reduce the copper as much as practical in the excess regenerated

acid solution, or the regenerated acid solution from the copper tanks No. 3, so that the acid solution will be rather low in copper when it is applied to the original ore to dissolve the acid soluble copper from the ore. It is preferred, therefore, when necessary, to combine the foul, rich, and nearly neutral copper solution obtained from leaching the original ore with the impure regenerated acid solution from the copper tanks, and then electrolyzing the mixed solution to impoverish or strip it of copper to the desired extent, in the copper stripping tanks. This may be done effectively by applying sulphur dioxide from the roasting furnace to the foul copper solution to reduce ferric iron to the ferrous condition, and then electrolyzing the foul copper solution, reduced in acid, to deposit the copper. In this way, from two to three pounds of additional acid may be regenerated, per pound of copper deposited from the foul solution. The mixing of the solutions reduces the acidity, and permits of more effective reduction of the ferric iron, and makes practical quite close stripping of the copper from the solution.

The cathodes from the foul solution copper stripping tanks will usually be quite impure. They may be refined by using them as soluble anodes in the practically pure copper solution in the copper tanks No. 1. The cathodes produced in copper tanks No. 1 and No. 2 will be of great purity, and the cathodes in Copper tanks No. 3 can be made so by depositing from a solution which is not too lean in copper, and then stripping the copper in the copper stripping tanks.

If the copper in the rich foul solution obtained from leaching the original ore is deposited electrolytically, the remaining very lean solution may be treated with hydrogen sulphide to precipitate the copper as sulphide, and the barren solution wasted. The wasted solution would about equal in amount the fresh water added for water leaching the roasted concentrate, plus that necessary or desirable to wash soluble copper from the ore, preparatory to flotation or gravity concentration.

When the copper concentrate permits of separation into a high grade and a low grade concentrate, certain advantages will result by the treatment described. The roasting of copper concentrate to get a high extraction of the copper is by no means simple. It requires care, especially if a high percentage of the copper is to be made water soluble without making a large amount of water soluble iron. If the larger portion of the copper can be concentrated into a relatively small amount of high grade copper concentrate, the high grade concentrate can be given the necessary care to get a high extraction of the copper and a pure electrolytic metal. By separating a small amount of high grade concentrate, the

treatment of the low grade concentrate is greatly simplified. There is no need of handling the low grade concentrate with the same care, either in roasting, leaching, or in the deposition of the copper, as if the high grade concentrate were mixed with it.

If the copper ore contains rare or precious metals worth recovering, the precious metals will be concentrated with the copper sulphide, and usually in about the same proportion. As applied to the specific case for illustration, about 83% of the precious metals will go with the concentrate and about 17% with the concentrator tailing; and if the concentrate is divided into a high grade concentrate and a low grade concentrate, 60% of the precious metals will be with the 1.5 tons of 50% copper concentrate, and about 40% of the precious metals will be with the 8.5 tons of 6.2% copper concentrate. The treatment of the copper concentrate leached residue to recover the precious metals will depend on their value and on the extent to which the copper can be extracted from the roasted concentrate, previous to leaching for the precious metals. If the residue can be cyanided, that would probably be the best treatment for the recovery of the precious metals, but the cyaniding of copper leached residue will depend almost entirely on the copper extraction. There should not be any difficulty in getting a sufficiently high extraction of the copper in the low grade concentrate to make cyaniding of the residue practical, and with the double roasting and leaching of the high grade concentrate, all of the leached copper concentrate residue should be made amenable to cyanidation, if the precious metal content is of sufficient value to warrant the treatment of all the concentrate residue. If, however, the precious metal values are so small as not to warrant a general treatment for their recovery, the high grade concentrate can be treated alone for the recovery of the precious metals. Of the 3,000 pounds of copper in the 100 tons of original ore 1500 pounds, or half of the copper, will be in the 1.5 tons of high grade concentrate, and consequently also about half of the precious metals. If the high grade concentrate, through roasting and leaching is reduced in weight by 60%, the leached 1.5 tons of roasted high grade concentrate residue will weigh about 0.6 tons, and will contain all of the precious metals originally in the high grade concentrate. Even if the precious metal content in the original ore is very low, it would still probably be highly profitable to recover the precious metals from the roasted and leached high grade concentrate residue. If, for example, the original ore assayed ten cents in gold and silver, and 50% is concentrated in the high grade concentrate, the leached high grade concentrate residue would assay about \$8.33, which could be very

105  
90  
95  
100  
105  
110  
115  
120  
125  
130

profitably recovered. If cyaniding of the copper leached residue is for any reason impractical, chlorination can almost always be successfully employed.

5 If the roasted concentrate is first treated with water or with a very dilute acid solution, so that dissolved iron is precipitated from the solution, or soluble iron made insoluble by hydrolysis, the water soluble copper solution can be maintained quite low in soluble iron, but the precipitated or hydrolyzed iron in the leached concentrate will be dissolved by leaching with the dilute acid solution in which the acid is in excess, to dissolve the acid soluble copper from the concentrate. 10 The copper can be readily deposited from the water soluble copper solution, very low in iron, and if the small amount of ferric iron formed by the electrolysis is effectively reduced, the re-solution of the deposited copper can be closely controlled. This makes possible a wide variation in current density for effective electrolysis. Where the cost of electricity is largely governed by peak loads 15 the electrolysis can be carried out at a maximum current density during the day when the load factor for other uses is low, and at a minimum current density when the load on the power plant for other purposes approaches and recedes from the peak load. 20 This will make possible, in many cases, a low, or minimum cost for power for copper deposition, and the power cost, in any electrolytic process, is of prime importance.

25 On the other hand, the acid soluble copper will be accompanied by high soluble iron. The stronger acid, will dissolve the acid soluble iron and also the iron precipitated from the water soluble copper solution, and that 30 hydrolyzed in the concentrate. The acid soluble copper solution will therefore be high in iron, but this iron can be controlled, in the deposition of the copper, with sulphur dioxide or copper sulphide, as described, and as 35 set forth more fully in my Patent No. 1,483,056, Feb. 5, 1924.

The water soluble copper and the acid soluble copper, should be deposited in different electrolytic circuits. The iron in the acid 40 soluble copper solution may be an advantage, because some of the iron may be regenerated with the acid in the deposition of the copper, and the regenerated acid and ferric iron solution may be applied to oxidized copper ore, 45 where both the acid and the ferric iron act as solvents for the copper.

The regulation of the current density of varying intensity, and cyclically regulated for the 24 hours per day according to the 50 assumption of power extraneous to the copper deposition circuit, will be more or less dependent on the absence of ferric iron in the electrolyte. Ferric iron dissolves copper more or less proportional to its presence in 55 the electrolyte. A low current density, which

would be used when the consumption of power for other purposes is at its peak, would be questionable economy if the ferric iron in the electrolyte is high, on account of the re-solution of the deposited copper; but if the 60 ferric iron is low or maintained reduced, the re-solution of the copper is small and the loss in efficiency would not be appreciable. As a practical illustration, a cell room could be designed for a maximum current density of 70 15 amperes per square foot. During the peak load for other power uses the current density could be dropped to as low as 5 amperes per square foot, with a proportionate diminution of power. Intermediate regulations might be 75 made for 10 amperes per square foot. This equalization of the power for all purposes of the power line or power plant so that the load would be very roughly constant for the full 80 24 hours, would make possible the acquisition of very cheap power, especially water power, where the load can be maintained practically constant for the full 24 hours at about the same cost as a greatly varying load delivering 85 much less power for the full 24 hours. 90

I claim:

1. A process comprising, treating copper ore to separate a high grade and a low grade copper concentrate, roasting the high grade concentrate, leaching the roasted high grade 95 concentrate to extract a portion of the copper, mixing the leached roasted high grade concentrate residue with the low grade concentrate, roasting the mixture, and leaching the roasted mixture to extract the copper. 100

2. A process comprising, treating copper ore to separate a high grade and a low grade copper concentrate, roasting the high grade concentrate, roasting the low grade concentrate, leaching the roasted high grade concentrate, electrolyzing the resulting copper solution to deposit the copper and regenerate acid, and leaching the roasted low grade concentrate with said acid solution. 105

3. A process comprising, treating copper ore to separate a high grade and a low grade copper concentrate, roasting the high grade concentrate, leaching the roasted high grade concentrate to extract a portion of the copper, adding the leached residue of the roasted 110 high grade concentrate to the low grade concentrate, roasting the low grade concentrate, electrolyzing the copper solution obtained from leaching the high grade concentrate to deposit the copper and regenerate acid, and leaching the roasted low grade concentrate 115 with said regenerated acid solution. 120

4. A process comprising, treating copper ore to separate a high grade and a low grade copper concentrate, roasting the high grade concentrate, roasting the low grade concentrate, leaching the roasted low grade concentrate to extract a portion of the copper, leaching the roasted high grade concentrate 125 130 with the copper solution obtained from leach-

ing the roasted low grade concentrate, and electrolyzing the resulting copper solution to deposit the copper as the electrolytic metal.

5. A process comprising, treating copper ore to separate a high grade and a low grade copper concentrate, roasting the high grade concentrate to make a portion of the copper water soluble, roasting the low grade concentrate to make a portion of the copper water soluble, leaching the roasted low grade concentrate to extract a portion of the copper, leaching the roasted high grade concentrate with the copper solution obtained from leaching the roasted low grade concentrate, electrolyzing the resulting relatively pure copper solution to deposit the copper and regenerate acid, applying the regenerated acid solution to the partly leached roasted low grade copper concentrate to extract more copper, and electrolyzing the resulting relatively impure copper solution separately from the relatively pure copper solution to deposit the copper.

6. A process comprising, treating copper ore to separate a high grade and a low grade copper concentrate, roasting the high grade concentrate to make a portion of the copper water soluble, roasting the low grade concentrate to make a portion of the copper water soluble, leaching the roasted low grade concentrate to extract a portion of the copper, leaching the roasted high grade concentrate with the copper solution obtained from leaching the roasted low grade concentrate, electrolyzing the resulting copper solution to deposit the copper and regenerate acid, and applying the regenerated acid solution to the roasted low grade concentrate to extract another portion of the copper.

7. A process comprising, treating copper ore to separate a high grade and a low grade concentrate, roasting the high grade concentrate, roasting the low grade concentrate, leaching the high grade concentrate to extract the copper, electrolyzing the resulting copper solution to deposit the copper and regenerate acid, leaching the low grade concentrate with the regenerated acid solution, electrolyzing the resulting copper solution to deposit the copper and regenerate acid, and dissolving the copper in the ore in its oxide combinations with the regenerated acid solution.

8. A process comprising, treating copper ore to separate a high grade and a low grade copper concentrate, roasting the high grade concentrate, roasting the low grade concentrate, leaching the high grade concentrate to extract a portion of the copper, electrolyzing the resulting copper solution to deposit the copper and regenerate acid, returning a portion of the regenerated acid solution to the roasted high grade concentrate, and leaching the roasted low grade concentrate with another portion of the regenerated acid solution.

9. A process comprising, roasting copper concentrate to make a portion of the copper water soluble, leaching the roasted concentrate to extract the water soluble copper, electrolyzing the resulting relatively pure copper solution to deposit the copper and regenerate acid, then leaching the roasted concentrate with the relatively pure regenerated acid solution to extract the remaining copper, electrolyzing the resulting relatively impure copper solution separately from the relatively pure copper solution to deposit the copper and regenerate acid, and then applying the relatively impure regenerated acid solution to copper ore to extract the copper naturally occurring in its oxide combinations.

10. A process comprising, roasting copper concentrate to make a portion of the copper water soluble and a portion acid soluble, leaching the concentrate to extract the water soluble copper, electrolyzing the resulting water soluble copper solution to deposit the copper and regenerate acid, then leaching the concentrate with the regenerated acid solution to extract the acid soluble copper, then in a separate electrolytic circuit alternately subjecting the resulting impure copper solution containing salts of iron to electrolysis and to the action of sulphur dioxide to deposit the copper and regenerate acid, and then leaching copper ore with the resulting impure regenerated acid solution to extract the copper naturally occurring in the ore in its oxide (including carbonate and silicate) combinations.

11. A process comprising, roasting copper concentrate to make a portion of the copper water soluble and a portion acid soluble, leaching the concentrate to extract the water soluble copper, electrolyzing the resulting water soluble copper solution to deposit the copper and regenerate acid, then leaching the concentrate with the regenerated acid solution to extract the acid soluble copper, electrolyzing the resulting impure copper solution in a separate electrolytic circuit to deposit the copper and regenerate acid, leaching copper ore with the resulting impure regenerated acid solution to extract the copper therefrom in its oxide (including carbonate and silicate) combinations, precipitating the copper from the resulting lean and foul copper solution, and returning the resulting barren solution to the ore to extract more copper in its oxide combinations.

12. A process comprising, roasting copper concentrate to make a portion of the copper water soluble and a portion acid soluble, leaching the concentrate to extract the water soluble copper, electrolyzing the resulting water soluble copper solution to deposit the copper and regenerate acid, then leaching the concentrate with the regenerated acid solution to extract the acid soluble copper, electrolyzing the resulting impure copper solution in a separate electrolytic circuit to de-

5 posit the copper and regenerate acid, leaching copper ore with the resulting impure regenerated acid solution to extract the copper from the ore in its oxide (including carbonate and silicate) combinations, electrolyzing the resulting foul copper solution or a portion thereof to deposit the copper and regenerate acid and ferric iron, and returning the resulting acid solution to the ore to extract more copper therefrom in its oxide combinations.

10 13. A process of treating mixed oxide and sulphide copper ore comprising, treating the ore to separate a sulphide concentrate, roasting the sulphide copper concentrate to make a portion of the copper water soluble and another portion acid soluble, leaching the roasted concentrate to dissolve the water soluble copper, then leaching the roasted concentrate to extract the acid soluble copper, separately electrolyzing the water soluble copper solution and the acid soluble copper solution to deposit the copper and regenerate acid, applying the regenerated acid solution from electrolyzing the water soluble copper solution to extract the acid soluble copper in the roasted concentrate, and applying the acid solution obtained from electrolyzing the acid soluble copper solution to the ore or concentrator tailing to dissolve the copper therefrom in its oxide combinations.

15 14. A process of treating mixed oxide and sulphide copper ore comprising, grinding the ore, adding a dilute acid solution to the finely ground ore to extract the copper therefrom in its oxide combinations, separating a portion of the resulting copper solution from the leached ore, subjecting the leached ore to flotation or gravity concentration to separate a sulphide copper concentrate, roasting the concentrate, leaching the roasted concentrate to extract the copper, electrolyzing the resulting copper solution to deposit the copper and regenerate acid, mixing the regenerated acid solution still containing some copper with the copper solution obtained from leaching the finely ground ore and electrolyzing the resulting mixed solution to deposit copper and regenerate acid, and applying the resulting regenerated acid solution to the finely ground ore to extract the copper therefrom in its oxide combinations, and repeating the cycle.

20 15. A process comprising, treating copper ore containing precious metals to separate a high grade and a low grade concentrate, roasting the high grade concentrate, leaching the roasted high grade concentrate to extract a portion of the copper, mixing the copper leached roasted high grade residue with the unroasted low grade concentrate, roasting the mixture, leaching the roasted mixture to extract the copper, and leaching the copper leached mixture residue to extract the precious metals.

25 16. A process comprising, treating copper

ore containing precious metals to separate a high grade and a low grade concentrate, separately roasting and leaching the high grade and the low grade concentrate to extract the copper, and treating the copper leached high grade concentrate residue to recover the precious metals.

30 17. A copper extraction process comprising, treating copper ore to separate a high grade and a low grade concentrate, separately roasting the high grade and the low grade concentrate, leaching one of the roasted concentrates to extract a portion of the copper as a relatively pure and relatively rich copper solution, then leaching the roasted concentrates to extract the remaining copper as a relatively impure copper solution, precipitating the copper from the relatively rich and relatively pure copper solution in one electrolytic circuit, and precipitating the copper from the relatively impure copper solution in another electrolytic circuit.

35 18. A copper extraction process comprising, roasting copper concentrate to make a portion of the copper water soluble and a portion acid soluble, leaching the roasted concentrate to extract a portion of the copper as a relatively pure and relatively rich copper solution, then leaching the roasted concentrate to extract the remaining copper as a relatively impure copper solution, precipitating the copper from the relatively pure and relatively rich copper solution in one electrolytic circuit, and precipitating the copper from the relatively impure copper solution in another electrolytic circuit.

40 19. A process comprising, treating copper ore to separate a high grade and a low grade concentrate, separately roasting the high grade and the low grade concentrate, separately leaching the roasted high grade and the low grade concentrate and electrolyzing the resulting copper solution to deposit the copper, and transferring the richer and purer portion of the copper solution from leaching the low grade concentrate to the high grade concentrate leaching and electrolytic circuit and transferring the leaner and fouler portion of the copper solution from leaching the high grade concentrate to the low grade concentrate leaching and electrolytic circuit.

45 20. A copper extraction process comprising, treating copper ore to separate a high grade and a low grade concentrate, roasting the low grade concentrate to make a portion of the copper water soluble and a portion acid soluble, separately roasting the high grade concentrate, leaching the roasted low grade concentrate to extract the water soluble copper as a relatively rich and relatively pure copper solution, then leaching the roasted low grade concentrate to extract remaining acid soluble copper as a relatively impure copper solution, treating the relatively rich and relatively pure copper solution with the

roasted high grade copper concentrate and electrolyzing the solution to deposit the copper, and separately precipitating the copper from the relatively impure copper solution.

- 5 21. A process comprising, treating copper ore to separate a high grade and a low grade copper concentrate, roasting the high grade concentrate, leaching the roasted high grade concentrate to extract a portion of the copper, 10 electrolyzing the resulting copper solution in one electrolytic circuit, mixing the partly leached roasted high grade concentrate residue with the low grade concentrate, roasting the mixture, leaching the roasted mixture to 15 extract the copper, and electrolyzing the resulting copper solution in another electrolytic circuit.

22. A process comprising leaching mixed oxide and sulphide copper ore with an acid 20 solution to extract the oxidized copper, subjecting the leached residue to flotation or gravity concentration to separate a high grade and a low grade concentrate, separately roasting the high grade and the low grade 25 concentrate, leaching the high grade concentrate to extract the copper, electrolyzing the resulting relatively pure and relatively rich copper solution to deposit the copper and regenerate acid, leaching the roasted low grade 30 concentrate with the regenerated acid solution to extract the copper, separately electrolyzing the resulting relatively impure copper solution to deposit the copper and regenerate acid, and applying the resulting relatively 35 impure regenerated acid solution to the mixed oxide and sulphide copper ore to dissolve the copper therefrom in its oxidized combinations.

23. A process comprising, leaching copper 40 ore to extract the copper, precipitating soluble iron from a portion of the copper solution, electrolyzing the solution low in salts of iron to deposit the copper and regenerate acid, redissolving the precipitated iron with the regenerated acid solution thus giving a copper 45 solution high in salts of iron, and separately electrolyzing the copper solution high in salts of iron.

24. A process comprising, leaching copper 50 per ore to extract a portion of the copper as a copper solution relatively low in salts of iron then leaching the ore to extract another portion as a copper solution relatively high in salts of iron, and separately electrolyzing the 55 solutions to deposit the copper.

25. A process comprising, treating copper ore to obtain a portion of the copper as a relatively pure copper solution and another portion as a relatively impure copper solution 60 containing salts of iron, electrolyzing the pure copper solution to deposit the copper and regenerate acid in one electrolytic circuit, and electrolyzing the impure copper solution containing salts of iron in another 65 electrolytic circuit to deposit the copper and

regenerate ferric iron, applying concentrated copper sulphide to the electrolyzed impure copper solution to reduce the ferric iron, and again electrolyzing the solution.

26. A process comprising, treating copper bearing material to obtain a portion of the copper as a copper solution low in soluble iron and another portion as a copper solution high in soluble iron, electrolyzing the copper solution low in soluble iron to precipitate the copper, and separately precipitating the copper from the solution high in soluble iron by alternately subjecting the solution to reduction and electrolysis. 70

27. A process comprising, treating copper bearing material to obtain a portion of the copper as a copper solution low in soluble iron and another portion as a copper solution high in soluble iron, electrolyzing the copper solution low in soluble iron to precipitate the copper, and separately precipitating the copper from the solution high in soluble iron by alternately subjecting the solution to reduction and to electrolysis with insoluble anodes. 75

WILLIAM E. GREENAWALT.

80

85

90

95

100

105

110

115

120

125

130